

A. F. SHORE.  
CASE HARDENING OF STEEL.  
APPLICATION FILED MAY 17, 1911.

1,072,660.

Patented Sept. 9, 1913.

Fig. 1



Fig. 2



Fig. 3



WITNESSES:

Orvin D. Dury  
Joseph Kleinier

INVENTOR

Albert F. Shore,  
BY  
Geo. A. Hoffman  
ATTORNEY

# UNITED STATES PATENT OFFICE.

ALBERT F. SHORE, OF NEW YORK, N. Y.

## CASE-HARDENING OF STEEL.

1,072,660.

Specification of Letters Patent. Patented Sept. 9, 1913.

Application filed May 17, 1911. Serial No. 627,747.

To all whom it may concern:

Be it known that I, ALBERT F. SHORE, a citizen of the United States, residing at 226 West Twenty-fourth street, New York, in the county of New York and State of New York, have invented certain new and useful Improvements in Case-Hardening of Steel, of which the following is a full, clear, and exact specification.

This invention relates to a process of case-hardening steel, and especially such articles as armor-plate, gun projectiles, and large gear teeth, as well as parts of machinery subjected to such constant use and vibration that methods of case-hardening now known to the art have proved unreliable, because of their inability to prevent portions of the hardened surface from flaking or peeling off; and the main object of the invention is to carburize a steel surface to such depths and in such a manner as to produce a relatively thick layer of carburized metal, which, when hardened, will remain permanently united with its softer backing under substantially all conditions of use.

I overcome the serious disadvantage just referred to by eliminating the flat cleavage plane between the hard and soft sections of the steel and providing instead an irregular cleavage surface between the two sections or strata of the steel, one such surface being formed by knob-like projections of the soft section extending upward a predetermined distance into the hard section, and thus providing an interlocking arrangement between the two sections, similar to plaster in wall lathing. This internal interlocking is due mainly to my process of carburization, the details of which will be set forth herein-after, as well as other features of my invention, all of which are shown in the accompanying drawings forming part of this application, and in which drawings—

Figure 1 illustrates the surface of a plate covered at intervals with protective coatings; Fig. 2 is a cross-section, illustrating the effect of the coatings on the penetration of carbon and shows the condition of the surface section of the plate at the end of a first carburizing period, and Fig. 3 is a cross-section showing the extent of the carbon penetration after the removal of the coatings and at the end of a second carburizing period.

The drawings illustrate a specific embodiment of my invention, in which the first

step in the process employed is to protect certain portions of the surface of the plate 1, underneath which an irregular cleavage surface is to be formed, from the carburizing agent, by suitable coverings, such as 2, which may be disk-like in form, of copper, enamel, cement, or the like, and of any desired size or shape. In said process the plate 1 is then subjected to a first carburizing action by any suitable carburizing agent and carburized to the desired depth as indicated in the carburized zone 3. The next step in said process is to remove the coverings 2, thus exposing the hitherto protected portions of the plate; after which the entire surface of the plate is then subjected to a second carburizing action, which is continued until the desired depth of carburization has been obtained, as indicated by the carburized zone 3', Fig. 3, which is sectioned to distinguish it from the uncarburized zone 1'. The next step of said process is to thoroughly harden the plate by chilling, in any usual manner. By this process an irregular cleavage surface will be produced which will separate the hard and soft zones or sections of the plate and will outline interlocking means such as projections 5, fitting into corresponding sockets, for holding said sections together in the form of a single unitary body. When a shell or projectile comes in contact with the surface of armor-plate as heretofore made, the usual result is the shattering of the point or nose of the shell, while the hardened surface of the plate is simultaneously crushed and large flakes stripped from the surface of the plate in all directions, thus exposing the soft section thereof. The shell or projectile, having an excess of penetrating energy, continues to cut into and through the soft section or back of the plate, punching out the same, as in a punching machine, and explodes in the interior of a vessel. The old type of armor-plate is thus seriously defective, in that the hardened section is detached from the soft section as above described; and frequently without warning large portions of the hardened section peel or flake off from the soft section of the plate because of internal stress resulting from heat treatment when the plate is made, and often augmented by extreme atmospheric changes.

According to my invention, it will be seen that the hardened section opposes lateral

resistance also to the separation of the two zones and this prevents its detachment from the soft section of the plate, which results from the impact of shells or projectiles, or from other external or internal causes. Thus fractures are not only localized, because of the irregular cleavage plane, but penetration of the plate by shells or projectiles is prevented, and the destruction or explosion of the latter on the exterior of the vessel is assured.

Applied to machine parts, spotting with an atomizer may take the place of the disks or coatings shown in Fig. 1, and here, as in the case of armor plates, the hardening is produced by the carburizing and chilling methods above described.

It will be understood that various modifications may be made in my invention without departing from the spirit and scope thereof.

What I claim is:

1. In a process of case-hardening steel, subjecting to direct shallow carburization inward through the face thereof portions of the surface of the steel to be treated, and subjecting to deep carburization the remainder of said surface.

2. In a process of case-hardening steel, subjecting to direct shallow carburization inward through the face thereof a multiplicity of relatively small areas of the surface of the steel to be treated, and subjecting to deep carburization the remainder of said surface.

3. In a process of case-hardening steel, subjecting to direct shallow carburization inward through the face thereof a multiplicity of relatively small areas of the surface of the steel to be treated, subjecting to deep carburization the remainder of said

surface, and then hardening the carburized layer so formed.

4. In a process of case-hardening steel, subjecting the surface and layer to be carburized to carburization in two different stages in one of which portions of the surface to be carburized are protected from, and in the other of which they are exposed to, direct carburization.

5. In a process of case-hardening steel, subjecting the surface and layer to be carburized to two different carburizing actions during one of which portions of the surface to be carburized are covered with carbon-resisting material and during the other of which said portions are not so covered.

6. In a process of case-hardening steel, covering portions of the surface of the steel to be treated with carbon-resisting material, carburizing the unprotected portions of said surface to the desired depth, removing the carbon-resisting material, and then subjecting the entire surface to a second carburizing action for the desired length of time.

7. In a process of case-hardening steel, covering portions of the surface of the steel to be treated with disks of carbon-resisting material, carburizing the unprotected portions of said surface to the desired depth, removing the carbon-resisting material, and then subjecting the entire surface to a second carburizing action for the desired length of time.

In testimony whereof, I affix my signature, in presence of two witnesses.

ALBERT F. SHORE.

Witnesses:

WILLIAM F. SHORE,  
CHARLES P. SHORE.